

## UNITED STATES PATENT OFFICE

RICHARD ELSSNER, OF JOHNSON CITY, TENNESSEE, ASSIGNOR TO AMERICAN GLANZSTOFF CORPORATION, OF NEW YORK, N. Y., A CORPORATION OF DELAWARE

## YARN WITH EVEN SHRINKAGE

No Drawing.

Application filed July 9, 1931. Serial No. 318,479.

My new invention has to do with a novel method for preventing the uneven shrinkage of artificial filaments.

More particularly, my invention has to do with the prevention of uneven shrinkage occasioned by drying cakes of artificial filaments produced by the pot spinning or centrifugal process.

In the pot spinning or centrifugal method for producing artificial filaments, a cellulosic solution is made up and extruded by pressure through fine orifices into a setting medium from whence it is carried over guiding means to a rapidly revolving receptacle which collects and twists the groups of filaments which are led thereinto. This receptacle or pot throws the filaments against its sides and thus builds up a cake of filaments which, when a sufficient number of filaments 20 has been bunched, is removed therefrom. These cakes are then washed, dried, and otherwise treated. As a result of these treatments the filaments are no longer tightly caked but are comparatively loosely wound. 25 The cakes may be dried either by skeining the cakes or drying the yarn directly in cake form. The drying in the cake form may be done by drying from the inside or from the outside but drying in one direction only, or 30 the yarn is dried from both sides towards the middle of the cake. If the yarn is dried from the outside towards the center the outer lying filaments tend to shrink before the inner filaments and thus an uneven shrinkage of the 35 yarn in the cake results. Similarly, if the yarn is dried from the inside toward the outside an uneven shrinkage results. I have discovered a method whereby this uneven shrinkage may be overcome.

According to my new method the cakes are taken from the centrifugal pot, washed, or otherwise treated, and then dried, for example, from the outer to the inner side. The cake is then wet again and dried now 45 from the inner to the outer side. This double drying has the unusual result that the filaments first shrink from the outside to the inside thus partially shrinking the middle 50 filaments, and then shrink from the inside to the outside thereby completing the shrinking of the middle filaments and equalizing the shrinking of both the outer and inner sides. This two step drying, wetting, and 55 drying process results in a cake of filaments

which is thoroughly dried and which possesses even shrinkage.

One means whereby the double drying may be accomplished may be described as follows: The cake of yarn is removed from the spinning pot, and the outside surface thereof covered with a water and air tight covering. This cake is then subjected to a drying from the inner to the outer layer of filaments. Then the outer cover is removed; the cake is 65 wet with water; and the water and air tight cover placed about the inner surface of the cake. The drying is then repeated this time from the outer to the inner layer of filaments.

As an alternative method, I have found 70 it feasible to dry, for example, from the inner to the outer side, reverse the loose cake of filaments, that is, turn the now loose cake inside out, and dry again in the same direction.

It should be understood that when the outer layer is covered as set out above, the top and bottom surfaces of the cake may be similarly protected by flaps extending from this cover.

Having now fully set forth my new invention as required by the patent statutes, what I desire to claim is:

1. A process for producing even shrinkage of filaments produced by the pot spinning process, which comprises drying the cake from the outside thereof, wetting the cake, and then drying the cake from the inside thereof.

2. A process for drying artificial filaments 90 produced by the pot spinning process which comprises wrapping the outside of the cake with an air and water tight covering, drying the cake from the inside, removing the wrapping, wetting the cake, then wrapping 95 the inside of the cake with an air and water tight wrapper, then drying the cake from the outside.

3. In a process for handling spun cakes of artificial filaments, the steps of wrapping the 100 outside of a wet cake produced by the centrifugal process with a covering, drying the cake by applying the drying medium to the uncovered portion of the cake, removing the covering, rewetting the cake, wrapping the 105 inside portion of the cake with a covering, and drying by applying the drying medium to the uncovered portion of the cake.

In testimony whereof I affix my signature.

RICHARD ELSSNER. 110